

July 15, 1924.

1,501,338

A. M. HENRY

ROTARY CASTING

Filed Oct. 9, 1923

3 Sheets-Sheet 1



INVENTOR

Augustus M. Henry

July 15, 1924.

1,501,338

A. M. HENRY

ROTARY CASTING

Filed Oct. 9, 1923

3 Sheets-Sheet 2



Augusto M. Henry *INVENTOR*

July 15, 1924.

1,501,338

A. M. HENRY

ROTARY CASTING

Filed Oct. 9, 1923

3 Sheets-Sheet 3



Figs. 8



Figs. 7



INVENTOR

Augustus M. Henry

Patented July 15, 1924.

1,501,338

# UNITED STATES PATENT OFFICE.

AUGUSTUS M. HENRY, OF BROOKLYN, NEW YORK.

## ROTARY CASTING.

Application filed October 9, 1923. Serial No. 667,524.

*To all whom it may concern:*

Be it known that I, AUGUSTUS M. HENRY, a citizen of the United States, and a resident of the city of New York, borough of Brooklyn, in the county of Kings and State of New York, have invented certain new and useful Improvements in Rotary Castings, of which the following is a full, clear, and exact description.

10 The present invention relates to the art of rotary or centrifugal casting; and aims to provide a novel and valuable method of and apparatus for (a) rapidly and economically producing ferrous castings of 15 ring or even sleeve and other forms, while insuring (b) that such castings always will include, merely as the result of the casting operation itself, a particular metallurgical characteristic essential if not highly desirable in various industries.

The prime object of the present invention, in the latter regard, is to form the casting by the centrifugal method and at the same time treat the casting as it solidifies so that 25 the same will be case-hardened where contacted by all or some of the walls of the mold cavity.

Another object is to provide a method and apparatus as above, wherein the mold is 30 formed of or has its cavity lined or faced with a material which is practically as inexpensive and as easy to machine smoothly and nicely to shape, as is iron or steel; which material is made up of masses of 35 granular components as tenaciously cohesive as iron or steel but yet a material adapted to be machined or pressed into a mold or mold-part not having the liability of a similar iron or steel part to crack, chip and dis- 40 tort from molecular "growth" as the result of repeated heat-shocks, i. e., as the result of repeated casting operations,—thus truly providing a permanent rotary mold; which material may be absolutely depended on 45 to give up some of its own content to the contacting superficies of the molten metal impacted against the mold by centrifugal force at each casting operation but not enough thereof to preclude the mold from 50 being employed for making a great number of castings having only absolutely negligible variations of contour, bulk and weight, such donated content constituting the carbonaceous matter for co-acting with the heat 55 of the metal incident to its molten state, thereby to predetermine that the casting

when ejected from the mold and merely allowed to cool on the floor of the foundry will be case-hardened according to the invention; and which material will not, like 60 iron or steel, chill the casting as an iron or steel mold always does. Such a material, I have discovered, is carbon, preferably 65 densely compacted; such for instance, as is known as gas carbon and as is used for making carbon-electrodes for electric arc lamps or for making the commutator brushes for dynamos, motors and the like.

To explain the practical and salient distinctions between a chilling and a case-hardening of a ferrous casting: When such a casting is chilled, the term is used, herein and indeed generally, to describe what happens to the superficial layer of a fairly large mass of cast iron when such mass is cast and such layer is solidified against a metal mold. Said layer, obviously, has the same carbon content as the rest of the casting, except that the layer has its carbon in the combined form and the carbon of the mass 80 of the casting underlying such layer is largely or wholly graphitic. On the other hand, case-hardening as hitherto practiced, has involved (a) the making, usually if not always in a sand-mold, of a soft iron casting, that is, a casting having therein a more or less uniform distribution of carbon largely or wholly in the graphitic form throughout; and (b) the application to the 85 superficies of such casting, some time after removal from the mold and generally some time after the casting has been permitted to cool, of a carbonaceous material, as powdered charcoal, and a simultaneous heating of the casting to a point where the outer 90 cuticle of the casting is converted into a high-carbon steel by the cementation process, or, in other words, to a point where the mere skin of the casting is chemically carburized and such skin becomes a hard, 95 strong case for the inner metal mass of the casting. Such case, obviously, has a different and greater carbon content than the rest of the casting; as contradistinguished from the conditions prevailing in a chilled casting, where, as stated above, the outer chilled 100 layer has the same carbon content as the inner mass of the casting, and, further, the carbon of the chilled layer is carbon in the combined form and so resulting in a layer 105 very brittle and of little toughness and absolutely no malleability.

As a result of the fact, then, that the present invention provides a casting which is case-hardened merely, and not chilled as above, and a casting, moreover, having immediately below its case-hardened skin a uniformly close dense grain uninterrupted by air or blow-holes and deposits of slag and other impurities and with no portion harder or softer than another, which latter qualities are characteristic of all centrifugal castings, there is provided by the invention a method and apparatus particularly adapted, thereby to attain a special object of the invention, for making rapidly and economically, and in a permanent mold, cast-iron rims or tires for car, truck, locomotive and the like wheels for railroad rolling-stock, which tires will be, as the result of the casting operation solely, tougher than steel, practically as strong, and case-hardened at their track-engaging surfaces pursuant to the requirements of the present practice; while at the same time said tires will, on the one hand, be unhardened at their inner peripheral portions, to permit them to be easily machined to the characteristic stepped shape there required and, on the other hand, chilled in no part. The importance of the last statement cannot be too much emphasized; as a chilling of the portion of the casting formed against the mold walls, and hence a chilling of that part of a centrifugally cast rim subsequently to ride on and alongside the rail, provides always a railroad car-wheel which dare only be used with risk of serious accident. This is so because a chill is a hard external layer of the casting of such measurable thickness, and of such great brittleness, as to be extremely liable to originate a crack deep enough to extend itself into and through the entire thickness of the casting.

Another object of the invention is to provide, further, a casting apparatus of the rotary type particularly adapted for facilitating the method of the invention and for maintaining continuously the rapid production of case-hardened ferrous castings as above, and a comparatively simple and inexpensive apparatus whereby such speed of production may be so maintained and without endangering the integrity of the mold proper, preferably of carbon as above, by repeated removal of a completed casting at half-minute intervals or less.

Referring now to the accompanying drawings, wherein are illustrated a preferred embodiment of such apparatus, and an illustrative method of casting facilitated thereby according to the invention,

Fig. 1 is a side elevation of said embodiment, partially broken away and partially in section;

Fig. 2 is a transverse section, taken on the line 2-2 of Fig. 1;

Fig. 3 is a top plan view, on an enlarged scale, and looking down on the top of the mold as viewed in Fig. 1, according to the arrow 3 in said Fig. 1;

Fig. 4 is an enlarged detail view showing the mold-structure and its interior parts including the carbon mold pieces, this view being an axial section; and

Figs. 5, 6, 7 and 8 are diagrammatic views indicating successive operations and adjustments of the various parts in making and ejecting a casting.

Similar reference characters refer to similar parts throughout the several views of the drawings.

The apparatus shown includes a rotor-structure including a main driving or mold-supporting shaft 20, a mold structure to be hereinafter described, the armature, fixed on said shaft, of the driving motor 23, and certain other parts to be mentioned in a moment.

Shaft 20 is journalled on suitable anti-friction bearings in a central sleeve casing 24, which casing carries a plate-extension 25 on which the motor-stator or case is fixed.

This main casing 24 is, by oppositely offset stub-shafts one of which is shown at 26, mounted on a horizontal axis relative to a pair of A-frames 27 bolted at their feet to a concrete bed 28 and constituting the supporting framework for the rotor-structure.

The mold-structure includes a metal fixture 29, fixed on the upper end of shaft 20, and an upper metal fixture 30 held to rotation with the shaft 20 of the lower fixture 29 as follows: A cylindrical steel pin or stud 31 is set tightly in the lower fixture to protrude above the flat annular surface 29<sup>a</sup> of the latter and on which rests a similar surface 30<sup>a</sup> of the upper fixture; such pin being somewhat loosely received in a cylindrical recess 32 undercut in the surface 30<sup>a</sup>—there being provided three of such pins and recesses circumferentially of the mold, 120° apart.

The mold proper is established by annular blocks of carbon, of a suitable cross-sectional shape, that shown being the shape used when the apparatus is to be used for making track-wheel rims or tires; the carbon block 33 being seated as illustrated in lower fixture 29 and the block 34 being seated as illustrated in upper fixture 30. It will be noted that the lower fixture is annularly recessed beyond the central plain portion, such recess for receiving and centering the block 33 before securement of said block in place; and that the upper fixture is centrally conically cut away as indicated at 30<sup>b</sup>, for permitting the introduction of the molten metal, and also for providing a peripheral inner edge with which the inner periphery of block 34 may be registered to cen-

ter the latter before securing said block in place.

Attention is directed to the fact that the matching flat annular surfaces of the two metal fixtures for carrying the carbon blocks are at a lower level, with shaft 20 vertical and the mold uppermost, than the matching flat annular surfaces of said carbon blocks; which is a feature of considerable practical importance, for a reason to appear hereinafter.

The means for replaceably securing these blocks in place, includes the following provisions: Each block is provided outwardly of its main body with an offset peripheral flange, so that a metal clamping ring 35 may be applied over such flange of the block 33 and a similar ring 36 may be applied under such flange of the block 34. Through suitable matching apertures in these flanges and rings and into likewise matching tapped recesses in the upper fixture, are applied screws as indicated at 37; and so that these screws may be applied to clamp the rings 35 and 36 without danger of injuring the flanges of the carbon blocks engaged thereby, spring means as indicated at 38 are carried by the screws, such means including a plurality of alternately arranged slit or spring washers 30 and plane discs as shown. Preferably there are four of such screws and spring-equiments applied relative to each ring 35 and 36, spaced apart 90° circumferentially of the mold.

In order to insure further that the carbon block 34 will not shift relative to the metal parts of the mold, a plurality of shallow cylindrical recesses are cut in the fixture 30 opposite the portions of the carbon block 34 of maximum thickness, as indicated at 39, and in each of these recesses is nested, as illustrated, a split or spring washer of such dimensions and stiffness that when the block 34 is clamped to the mold by ring 35, a canted end of each washer in a recess 39 will bite into but not endanger the integrity of the block. Preferably there are six of such recesses and washers, spaced apart 60° circumferentially of the mold.

Means for axially separating the mold-fixtures 29 and 30, always parallelly, and different degrees as required, is provided as follows: Matching projections 29<sup>a</sup> and 30<sup>b</sup> are offset from the two fixtures, three of such projections being preferably provided, spaced apart 120° circumferentially of the mold. Over each projection 30<sup>b</sup>, upper mold-fixture 30 carries rigidly a plate or eave-projection 30<sup>c</sup>. Each projection 30<sup>b</sup> is provided with a smooth transverse bore of sufficient diameter to receive, with slightly more looseness than characteristic of the reception of the upper part of a stud 30 by its recess 32, a smooth cylindrical portion 40 of a shaft 65 S; and each projection 29<sup>b</sup> is drilled and

tapped in line with such bore to provide a tapped bearing for a screw 41 forming another portion of said shaft S. Said shaft S, at what may be termed its upper end, terminates in an enlarged head nested loosely 70 between the eave-projection 30<sup>c</sup> and projection 30<sup>b</sup> of the upper fixture. Said shaft carries, below its screw length 41, an elongate pinion or cylindrical rack 43; below this rack, a smooth cylindrical portion 44 75 is journalled in a suitable bearing in a disk 45 carried rigidly by main shaft 20, and below such disk, has a squared end to which may be applied a crank (not shown) to facilitate rotating the shaft S. The three 80 pinion racks 44 of the three shafts S all mesh with a spur gear 46 revolvably mounted by way of a suitable anti-friction bearing on said main shaft 20 but restrained from endwise movement relative to said main shaft. 85 It is obvious that by applying the crank last-mentioned to the squared lower end of the shaft S most conveniently accessible at the moment, at cessation of rotation of the rotor-structure at the conclusion of a casting operation, such crank may be turned to separate the two mold-fixtures 29 and 30, always parallelly, to the extent of separation desired,—such, for instance, as first to move such fixture apart as indicated in Fig. 6, next to move such sections apart as indicated in Fig. 8, and next to restore such sections to the close contiguity required for casting.

It is observed at this point that the flats of the A-frames 27 are obliquely inclined relative to their floor-plates or feet 27<sup>a</sup>, so as to insure that such flats will diverge in a downward direction when the floor plates 27<sup>a</sup> are bolted to the foundation bed 28; thus to permit the entire rotor-structure to be variously swung about the horizontal axis afforded by shafts 26 as shown in certain of the views last-mentioned and for a purpose which will be explained under "Operation" 100 hereinbelow.

In order to adopt the shafts S and their associated mounting and restraining devices, to act automatically to maintain the mold fixtures 29 and 30 in the close contiguity 105 above-mentioned, at all times during rotation of the mold, the following means is provided: Fixed on the portion 44 of each such shaft, is an offset ball 48 of sufficient weight and so disposed that its center of gravity is to one side of a straight line joining the axes of the associated shaft S and main shaft 20 when the mold-fixtures are manually brought to said contiguity, so that rotation of the mold-structure in the predetermined direction will always cause centrifugal force to act on these balls to cause them to apply turning moments to the shafts S 120 to hold the mold-fixtures close together.

Operation: With the mold-structure ro- 125

tating at the proper speed, preferably about an axis inclined 45° as shown in Fig. 1, a predetermined charge of molten metal is delivered to the mold as indicated by the arrow M; and in a few seconds a casting, of the cross-section indicated at C in Fig. 6, is set sufficiently to permit removal, and is also properly case-hardened where in contact with the carbon blocks 33 and 34. Rotation of the mold-structure having been stopped, such structure is rotated 45° about shafts 26 to dispose main shaft 20 as shown in Fig. 6. Thereupon, a workman applies his crank to the squared lower end of a shaft S, and turns such shaft and crank to separate the mold parts as shown in Fig. 6. Thereupon, the same or another workman, by the use of a suitable apparatus, appliance or fixture (not shown), slides into place a sheet metal shield 49 of any suitable outline, but preferably equipped with a layer of wood below the metal and a sheet of asbestos below the wood. Such shield is shown in place in Fig. 6, but with the three strata 25 just mentioned not delineated or marked off; it being understood, however, that the asbestos stratum corresponds in location with the lower bounding line of the shield as shown in this view, so as to preclude any possible chilling of the casting. It should be particularly noted that the matching flat annular surfaces of the two carbon blocks and of the two mold fixtures which mount the latter, are now at different levels 30 and so disposed relative to the now uppermost surface of the casting, that all parts of both blocks are protected against accidental danger by contact with the shield. With the parts thus arranged, the same or another workman next rotates such structure through 180° about shafts 26, to dispose the shaft 20 as shown in Fig. 7. Thereupon, the same or another workman applies his crank again to the squared end of a shaft S, and turns such shaft and crank to separate the mold parts as shown in Fig. 8. Whereupon, finally, with the shield suitably restrained against sliding movement relative to the mold, the casting is pushed or pulled 35 in the direction of the arrow 50, clear of the shield and the mold, and left to cool before being sent to the machine-shop for final finishing of its internal periphery.

As to the various processes of the present invention, these will be understood from the foregoing description of the apparatus shown in the drawings. In this connection, it is particularly to be understood that the present invention is of course not necessarily 40 to be limited to the making of rims or tires for car-wheels, of iron or steel, but may be applied to make other articles of annular cross-section, by which is meant either ring-shaped or sleeve-shaped articles, as, for instance, the so-called economizer sleeves for

boiler and superheater tubes and the like, journal boxes, mouths for steel tanks, and other articles to be investigated as articles of arcuate cross-section, for making, say, railway brake-shoes; as is indicated by the scope of the appended claims. 7

By the expression "cross-section" as used herein is meant a cross-section through the casting which would be taken, with the casting still unejected from the mold, in a plane perpendicular to the axis of rotation of said mold. 75

As to the apparatus shown, obviously variations may be freely resorted to within the scope of the said claims. 80

In said claims, wherever a mold or mold part is characterized as permanent, there is meant merely that said part is of a material or so constructed that the part will not be so injured by a single casting operation as to be useless for a second casting operation, as contradistinguished from a mold or mold part constructed or lined with ordinary foundry sand. 85

I claim:

1. A method of forming ferrous-metal articles which involves providing a mold having a cavity shaped to correspond with the predetermined external shape of a desired article, rotating the mold and thereafter admitting molten metal thereto, and thus utilizing centrifugal force to form a casting in said cavity while simultaneously applying to the portions of molten metal impacted by centrifugal force against the shaped parts of said mold cavity, a material to case-harden the resulting casting as to portions thereof formed by such shaped parts. 90

2. A method of forming ferrous-metal articles which involves providing a mold having a cavity shaped to correspond with the predetermined external shape of a desired article, rotating the mold and thereafter admitting molten metal thereto, and thus utilizing centrifugal force to form a casting in said cavity while simultaneously applying to the portions of molten metal impacted by centrifugal force against the shaped parts of said mold cavity a carbonaceous material. 95

3. The art of manufacturing ferrous-metal castings by the rotary casting method, which method involves providing a mold having a cavity formed by shaped pieces of carbon, rotating such mold and admitting molten metal to the rotating mold, and ejecting the casting after a sufficiently prolonged contact with the carbon elements of the mold to insure extra carburization of the parts of the casting so contacted with said carbon elements. 100

4. The art of forming ferrous-metal articles by the use of a permanent mold, which method involves providing a lining for said mold including a plurality of pre-shaped 105

100

105

110

115

120

125

130

blocks of gas-carbon to constitute the permanent mold proper, rotating the mold, and introducing molten metal into the rotating mold and treating such metal during solidification to case-harden the resulting casting in certain portions practically simultaneously with the creation of said casting.

5. The art of forming ferrous-metal articles by the use of a permanent mold, which 10 method involves rotating said mold and introducing molten metal into the mold and treating such metal during solidification to case-harden the resulting casting in certain portions practically simultaneously with the 15 creation of said casting.

6. The art of forming ferrous-metal articles by the use of a permanent mold, which method involves introducing molten metal into the mold and treating such metal during 20 solidification to case-harden the resulting casting in certain portions practically simultaneously with the creation of said casting, and removing said casting from the mold while still retaining sufficient heat to 25 insure self-annealing of the casting by such heat after removal of the casting from the mold, thereby to insure conversion to graphitic carbon of the combined carbon in any chilled portion of the casting.

30 7. In rotary casting apparatus, the combination of a rotary mold including a plurality of separable parts, means operable at will for bodily moving one of said parts relative to the other and also operable at 35 will for adjusting said parts to different degrees of separation, and centrifugally actuated means for locking said parts in predetermined adjacency during rotation of the mold.

40 8. In rotary casting apparatus, the combination of a rotary mold including a plurality of separable parts, and means operable at will for bodily moving one of said parts relative to the other and parallelly 45 thereto.

45 9. In rotary casting apparatus, the combination of a rotary mold including a plurality of separable parts, means operable at will for bodily moving one of said parts relative to the other, said means including 50 impositive adjusting means of the screw type, and centrifugally actuated means automatically operating to lock the mold parts securely in predetermined adjacency during 55 rotation of the mold.

55 10. In rotary casting apparatus, the combination of a rotary mold including a plurality of separable parts, means operable at will for bodily moving one of said parts relative to the other, said means including 60 an element revoluble about an axis different from the axis of rotation of the mold, and centrifugally actuated means for automati-

cally forcing said mold parts into close adjacency during rotation of the mold.

65 11. In rotary casting, the combination of a rotary mold including a plurality of axially separable parts, rotating means on which one of said parts is secured, operating means for axially separating the mold parts including an element bodily moved with the first-mentioned part during operation of said rotating means, and a foundation structure on which said rotating means is mounted for rotative adjustment about a 70 substantially horizontal axis.

75 12. In the art of making rotary castings of ring form by the use of a casting apparatus including a mold having a plurality of axially separable mold parts, journalling means for rotatably supporting the mold, means for separating the mold parts by different amounts, and a foundation structure on which said journalling means is rotatively adjustable about a substantially horizontal axis; the method of operating such apparatus, which comprises utilizing the mold to cast a ring-form article therein, thereupon, while said journalling means is positioned to support the mold thereabove, 80 separating the mold parts a certain amount, thereupon providing a sheet-like shield and inserting said shield between the mold parts and to overlie the casting, thereupon rotatively adjusting said journalling means to 85 dispose the mold therebelow, thereupon further separating the mold parts, and thereupon ejecting the cast article by moving the latter relatively to said shield and the mold in a direction substantially perpendicular to 90 the mold axis.

95 13. The method of producing ferrous metal articles from a molten charge which consists in forming a casting by centrifugal action in a shaping mold, and simultaneously applying case-hardening material to 100 parts shaped by the mold.

105 14. The method of producing ferrous metal articles from a molten charge which consists in forming a casting in a rotating shaping mold, and simultaneously applying case-hardening material to parts shaped by the mold.

110 15. The method of producing ferrous metal articles from a molten charge which consists in forming a casting by centrifugal action in a shaping mold, and simultaneously case-hardening parts shaped by the mold.

115 16. The method of producing ferrous metal articles from a molten charge which consists in forming a casting in a rotating shaping mold, and simultaneously case-hardening parts shaped by the mold.

AUGUSTUS M. HENRY.